

Patented July 8, 1941

2,248,100

# UNITED STATES PATENT OFFICE

2,248,100

## JEWEL MADE FROM GOLDEN COLORED ALLOYS

Otto Loebich, Pforzheim, Germany, assignor, by mesne assignments, to Chemical Marketing Company Inc., New York, N. Y.

No Drawing. Application March 11, 1939, Serial No. 261,309. In Germany March 25, 1938

2 Claims. (Cl. 63—2)

My invention relates to jewels made from gold-colored alloys, as for instance, rings, bracelets, necklaces, rimmings of spectacles, lorgnettes, opera-glasses and the like, which contain gold, copper and zinc as basic components and which may eventually contain also additional components, such as silver, metals of the platinum group, for instance, platinum, rhodium and palladium.

Jewels made wholly or partly from those alloys sometimes show the disadvantage to be subjected to a sudden destruction, for instance, by recomposition. These destructions may be disengaged also by external influences, as for instance, by the effect of corroding agents, such as perspiration. Hereby the co-operation of tensions which have been gone into the object by rolling, cold-drawing or the like, effect also the destruction which depends therefore on corrosions of tension.

Thorough investigations and experiments have shown that those disadvantages may be avoided by adding small amount of base metals, such as iron, to the alloys for the manufacture of the above mentioned jewels.

The metal which prevents the corrosion of tension may be added tel quel or in the form of a pre-alloy, for instance, with zinc or with gold.

Influences, as for instance, perspiration, which are able to disengage the dangerous tensions with alloys which do not contain iron, perhaps in the presence of the protecting metal iron act in such a way that they affect only the finest particles of the protecting metal by eventually dissolving traces of the same and thereby preventing direct attack of the precious metal alloy.

According to my invention the alloys for the manufacture of jewels may contain, for instance:

|        | Parts by weight |
|--------|-----------------|
| Gold   | 33 to 60        |
| Copper | 10 to 55        |
| Zinc   | 0.5 to 25       |

Protecting metal, such as iron or the like

|            |          |
|------------|----------|
| like       | 0.1 to 5 |
| preferably | 0.3 to 3 |

Furthermore they may contain, for instance, 1 to 30 parts of weight of silver and/or 1 to 15

parts of weight of the metals of the platinum group, such as palladium, platinum, rhodium, either alone or together.

The various alloys for the jewels according to my invention may be smelted in such a way that 5 100 parts of the alloys contain the desired components, for instance, gold, copper, zinc and iron, or, for instance, gold, copper, zinc, iron and silver, or, for instance, gold copper, zinc, iron and palladium, or, for instance, gold, copper, zinc, iron, silver, palladium, in such quantities that the amount of the single parts lies within the ranges mentioned above and that the sum of the single parts proves to be 100. If one desires to manufacture an alloy with a low grade of gold, for instance, 33 to 35 parts of gold will be used and then introduced a higher percentage of, for instance, copper whereby the additional metals are rated in such a way the value 100 will be attained. 15 20 With alloys richer in gold, for instance, 55 to 60 parts of gold will be used corresponding to smaller quantities of copper and so on.

The quantity of the white metals, such as silver, palladium and the like are rated in such a 25 way that the alloys show yet a gold color.

The alloy and the jewels made therefrom may be manufactured by well known methods.

An appropriate alloy for the manufacture of a jewel, for instance, a ring, a bracelet, a necklace, a rimming of a spectacle and the like may 30 have the following composition:

|        | Parts |
|--------|-------|
| Gold   | 333   |
| Copper | 390   |
| Zinc   | 185   |
| Silver | 82    |
| Iron   | 10    |

What I claim is:

1. A jewel made of a gold-colored alloy consisting of 33.3 parts of gold, 39.0 parts of copper, 18.5 parts of zinc, 8.2 parts of silver and 1.0 part of iron.

2. Gold colored jewel formed of an alloy containing 33 to 60 parts golds, 10 to 55 parts copper, 0.5 to 25 parts zinc, 1 to 30 parts silver and 0.1 to 5 parts iron.

OTTO LOEBICH.